

# UNITED STATES PATENT OFFICE.

CHRISTIAN BERGH BACKER, OF MONTREAL, QUEBEC, CANADA.

## METAL ALLOY.

1,341,774.

Specification of Letters Patent.

Patented June 1, 1920.

No Drawing.

Application filed December 30, 1918. Serial No. 268,923.

*To all whom it may concern:*

Be it known that I, CHRISTIAN BERGH BACKER, a subject of the King of Norway, and resident of the city of Montreal, in the 5 Province of Quebec and Dominion of Canada, have invented certain new and useful Improvements in Metal Alloys, of which the following is a full, clear and exact description.

10 This invention relates to a metal alloy, the main object of the invention being to produce a metal having a lower specific gravity than any of the light metal alloys at present in use, yet having equal if not 15 greater strength and toughness.

This new alloy consists of magnesium, aluminum and zinc, the proportion of magnesium being much greater than in any alloy heretofore produced. The proportions of 20 the metals in the alloy may vary approximately from 85% to 98% of magnesium, 1% to 14% of aluminum, and .5% to 6% of zinc, the exact composition of the alloy depending upon the use for which it is to be 25 applied. For instance, if a hard, close-grained metal is desired, the aluminum content is made comparatively high and the zinc content comparatively low, but the alloy will then have less ductility and strength.

30 For producing a hard and coarse-grained metal, both the aluminum and the zinc contents should be high, and approximately the same percentage, say 5%, of each should be used. For an alloy of great strength and

35 toughness, both the aluminum and zinc contents should be comparatively low, say not more than 5% aluminum and not more than 3% of zinc. I have also found that for certain purposes, it may be desirable to add

40 small percentages of one or more of the following metals, — calcium, copper and cadmium. For example, by adding 1.5% of copper to an alloy of magnesium, aluminum and zinc in approximately the proportions above stated, the strength and toughness of the alloy may be further increased, but the addition of copper has the disadvantage that the scrap metal can not then be as readily remelted as when magnesium,

50 aluminum and zinc only are used. Further, by adding approximately 2% of calcium to the magnesium, aluminum and zinc, the hardness of the alloy may be considerably increased without reducing its strength and the molten metal is also rendered more fluid

thereby. By adding a small percentage of cadmium, say less than 2%, neither the strength nor hardness of the alloy is affected, but I have found that the addition of cadmium lowers the melting point and makes 60 the alloy more fluid and easier to cast. While the addition of the metals, calcium, copper and cadmium in small quantities is found to be useful for the purposes stated, it is to be understood that they are not 65 essential to the quality of the metal produced in an alloy of magnesium, aluminum and zinc in the proportions mentioned.

As the alloy of metals constituting this invention consists of such a large percentage, 70 over 85%, of magnesium, it is necessary to melt the metals under special conditions to prevent the magnesium from being consumed by combustion. To accomplish this, the metals in the proportions specified are 75 placed in a crucible from which air is excluded. The molten metal may be then be run off and cast in special molds. The preferred method which I employ, however, is to cover the magnesium with a flux, then 80 melt the metal, and afterward add the proper proportions of aluminum and zinc until the mass is ready to cast in a mold.

This alloy has a very low specific gravity, 1.75 to 1.80; has great strength and toughness; has excellent wearing and anti-friction qualities as a bearing metal; and has a very high heat conductivity, nearly three times that of cast iron. This high heat conductivity, together with its quality of withstanding shock and vibration perhaps better than any other known metal, makes it particularly suitable for use in the manufacture of such parts as pistons and connecting rods for internal combustion engines. It has also 95 been found very suitable for bearings, gears and a great variety of other uses. Castings of this alloy may be bent as well as slightly extended without danger of breaking and by heating the casting to approximately 100 300° centigrade, it may be hammered and forged into almost any shape. The alloy may also be rolled and drawn under heat. It is not affected to any extent under atmospheric influences and, like aluminum, 105 becomes covered after a short time with a thin transparent coating of oxid which prevents further oxidation. This alloy takes a high polish and may be machined very easily and quickly, and in fact, may be 110

turned at speeds several times as high as that used in turning brass.

Having thus described my invention, what I claim is:—

- 5 1. An alloy consisting of not less than 85% and not more than 98% of magnesium, not less than 1½% and not more than 14% of aluminum and not less than ¼ of 1% nor more than 6% of zinc.
- 10 2. An alloy consisting of magnesium, aluminum and zinc, magnesium constituting

more than 85% of the metal, the aluminum more than 1½% and the zinc more than ¼ of 1% of metal by weight.

3. A low specific gravity alloy consisting of magnesium in the proportion of more than 85%, aluminum more than 1½% and zinc more than ¼ of 1% and adapted to be hardened by the addition of 2% calcium.

In witness whereof I have hereunto set my hand.

CHRISTIAN BERGH BACKER.